

April 12, 1960

K. VON HAKEN

2,932,563

PROCESS FOR REDUCING IRON ORES AT LOW TEMPERATURES

Filed Sept. 16, 1955

3 Sheets-Sheet 1

Fig. 1



Inventor:  
KURT VON HAKEN

B. E. Shlesinger  
attorney

April 12, 1960

K. VON HAKEN

2,932,563

PROCESS FOR REDUCING IRON ORES AT LOW TEMPERATURES

Filed Sept. 16, 1955

3 Sheets-Sheet 2



Fig. 2

Inventor:

KURT VON HAKEN

B. Schlesinger  
attorney

April 12, 1960

K. VON HAKEN

2,932,563

## PROCESS FOR REDUCING IRON ORES AT LOW TEMPERATURES

Filed Sept. 16, 1955

3 Sheets-Sheet 3



KURT VON HAKEN

Beklaagden  
attorney

1

2,932,563

**PROCESS FOR REDUCING IRON ORES AT LOW TEMPERATURES**

**Kurd von Haken, Murnau, Upper Bavaria, Germany, assignor of one-third to Johannes Bernhard Hahn, Munich, Germany**

Application September 16, 1955, Serial No. 534,685

Claims priority, application Germany October 13, 1954

3 Claims. (Cl. 75—26)

Starting from cinder of ores such as brown iron ores or taconites which can easily be cindered, e.g. hematite, goite, limonite, an oxidation process to brown magnetic  $\gamma$ - $\text{Fe}_2\text{O}_3$  is carried out. This oxidation has to be carried out at temperatures of from 330° C. to 270° C. with cooling; or else the  $\gamma$ -form becomes again the  $\alpha$ -form.

This  $\gamma$ -form can easily be magnetically separated from the gangue. A mechanical process in the disintegrator can be added.

During the reduction to iron by carbon monoxide, CO, already at a temperature of 160° C., a black iron coating is produced on the surface of this  $\gamma$ - $\text{Fe}_2\text{O}_3$ . The renewed reduction with CO takes place slowly. This can be explained by the slow escape of the developed  $\text{CO}_2$  from the micro-crystallites of the iron oxides.

The object of the invention is a process by which the grains or powder of iron oxide are brought into contact with the dust of soft coal containing bitumen or gas, by mixing and whirling them at reduction temperatures of from 350° C.—540° C.

Other iron oxides, iron ores or iron concentrates too are reduced by this reducing process at increasing temperatures to 640° C.

In order to continue the contact between coal and iron oxide the reduction is carried out under a perpetual whirling in a whirl layer process; simultaneously the burning of the coal or carbon monoxide is carried out at low temperatures without annealing.

It is already known that with higher temperatures than 330° C. by oxidation of cinder  $\text{Fe}_3\text{O}_4$  a loose black magnetic powder is obtained; but this product cannot be so easily and directly reduced from the micro-crystalline surface to iron as the brown  $\gamma$ - $\text{Fe}_2\text{O}_3$ . All parts of the product form a ball during the reduction with  $\text{Fe}_3\text{O}_4$  forming ferric oxide  $\text{FeO}$  while sintering.

In the drawings the reduction process is illustrated by diagram curves and by an embodiment of the furnace used for the execution of the process.

Fig. 1 shows diagram curves according to the co-ordinating system, the ordinates representing the temperatures and the abscissas the yield of pure iron;

Fig. 2 shows a whirl layer furnace for the execution of the process in vertical section through the whirl layers;

Fig. 3 shows the same whirl layer furnace as in Fig. 2 in vertical section rectangular to the section plane of Fig. 2.

In Fig. 1 the curves 1 and 2 are concerned with  $\alpha$ - $\text{Fe}_2\text{O}_3$ , a thin nonrotating layer of which has been treated with a gas containing 30% of CO for 15 or 30 minutes, at increasing temperatures. At a temperature of 400° C. the formation of  $\text{Fe}_3\text{O}_4$  can be observed. Just below 600° C. the production of ferric oxide  $\text{FeO}$  begins. Above the line A—B a stronger sinter zone is formed

2

under the influence of  $\text{FeO}$ , by which the reduction process is nearly impossible.

By a quick treatment with  $\gamma$ - $\text{Fe}_2\text{O}_3$  according to curve 3 in Fig. 1 one gets into this sintering zone within 15 minutes. Working for 30 minutes, curve 4, by slowly increasing the temperatures, a 100% pure iron powder will be obtained.

By treating  $\alpha$ - $\text{Fe}_2\text{O}_3$  in pellets with a whirl layer process at about 725° C. with the addition of CO, 40% pure iron was obtained in 7 minutes. By using loose  $\text{Fe}_3\text{O}_4$  the result was 50% pure iron.

These two experiments showed 3 or 4 times the speed of reduction of the non-whirled powder.

At the reduction of  $\gamma$ - $\text{Fe}_2\text{O}_3$  the use of the whirl layer process with addition of coal leads, within 10 minutes, according to the lower curve 6, to the production of iron at a temperature of about 540° C. By using a mixture with 50%  $\alpha$ - $\text{Fe}_2\text{O}_3$  this occurs at a temperature of 640° C. according to curve 5.

The vertical section of the whirl layer furnace 11 in Figs. 2 and 3 is divided into horizontal layers 12 the top layer contains dust separators 13 below the pneumatic introduction means 14 for  $\gamma$ - $\text{FeO}$  coming from the dust tank 15 with addition of gas above the uppermost layer of the distribution channels 16. The material introduced at the device 14 will be heated by the gas coming from below and oppositely directed to the falling down iron oxide powder meshed with gas (for 1 ton of iron 500 c.b. m. of gas), containing mainly CO,  $\text{CO}_2$ , H and N. CO will be burned at low temperature by the iron oxide to  $\text{CO}_2$ , so that it will not be lost.

The iron oxide material  $\gamma$ - $\text{Fe}_2\text{O}_3$  falls to the top whirl layers 12 and between those through the open intermediate spaces 17 to the lower whirl layers 12. Above each channel 16 a spaced cover with upwardly to the vertical central line of the channel inclined surfaces is disposed.

By a blowing engine 18 through the feed pipes 19 with throttle valves 20 which are opened at intervals by a moving endless chain 21 with an automatic driving mechanism carbon dust from dust tanks 22 with injectors 23 and gas 15 are advanced through the tubes 24 of the whirl channels 16 in one row of channels 16 after the other. The material is whirled up by gas stream. During the time between the intervals of opening the throttle valves 20 the material falls to the lower layers 12 through the intermediate spaces 17. Finally the reduced iron powder gets to the bottom through a tube cooler 25 where it is cooled below 100° C. and through a funnel 26 it is transported out of the furnace by any hydraulic means 34. Through a tube 27 bare annealing gas is introduced into the lower part of the furnace. Coal dust and grains of the material to be reduced will be introduced together with the gas pneumatically from tanks 14 through tubes 29 in the necessary quantity.

In the lowest layer 12 before the cooler 25 the material will be heated to a higher degree with gas flames 30, and soda and lime dust from tank 31 with injector 33 will be introduced together with gas through pipe 32. Thus a thin coating like glass is formed with ashes and the remainder of the gangue at about 700° C. on the surface of the iron dust. After its cooling the material is slightly ground in disintegrators and then separated in the magnetic separator as pure iron powder, or it will be brought directly to a foundry. The gas for heating and processing is produced in a special gas generator.

For the reduction about 12% carbon in the form of coal with respect to the weight of iron is necessary; if carbon is used in form of CO the double quantity of this gaseous carbon is necessary for the same weight of iron.

The reduction of other iron ores such as magnetite and pyrite residue can be carried out in such a way, that those are pelletised from powder with at least 30% of  $\gamma$ -Fe oxide together with coal dust and are afterwards burned in a blast furnace or low shaft furnace or cupola. The advantage is that the reduction process itself takes place at low temperatures and that only iron has to be melted besides the gangue without contents of oxygen. In that way the use of burning material is limited.

The continuous formation of iron starting from the surface is noticed, while brown  $\gamma$ -Fe<sub>2</sub>O<sub>3</sub> can be observed in the interior of the grains.

The process of gaining the brown  $\gamma$ -iron oxide for the production of pure iron, starting from cinder Fe<sub>3</sub>O<sub>4</sub> can only be carried out at falling temperatures from 350° C. to 270° C. It is preferred to use the same whirl layer furnace. The material has to be intensively cooled, as much heat will be released through this process.

The characteristic part of the invention consists in carrying out the continuous reduction on a basis of the contact of  $\gamma$ -Fe<sub>2</sub>O<sub>3</sub> with carbon dust at temperatures lying below the zone of sinter, line A—B, preferably at temperatures rising from 350° C. to 540° C.; by adding other iron oxides rising to about 640° C.

In this case the reduction takes place in about 10 minutes.

Impurities, as far as they enter the iron at those temperatures, have to be removed. Sulfides disappear during the magnetic separation. Phosphates only become useful for the process after a longer treatment at 650° C. with alkalines or alkaline bauxite residues and by washing out the tri-natriumorthophosphate, Na<sub>3</sub>PO<sub>4</sub>, before the producing of  $\gamma$ -Fe<sub>2</sub>O<sub>3</sub>.

Coal will not be absorbed by the iron at bare annealing conditions and at the low temperatures of the process.

The formation of small pellets with coal for facilitation of the furnace process, e.g., while manufacturing manganese (Mn) ores, is possible. At the final treatment of iron powder with about 0.1% of Na<sub>2</sub>CO<sub>3</sub> will be suitably added above 600° C. With the remaining amounts and ashes of coal it can easily be automatically ground and magnetically separated.

Well known materials which accelerate the reduction, such as wood dust, lime milk and water vapour, might be added. Especially at the end of the reduction water vapour is wanted for removing the carbonaceous coatings.

What I claim is:

1. A process for the production of pure iron from brown magnetic iron oxide,  $\gamma$ -Fe<sub>2</sub>O<sub>3</sub>, in which finely-divided  $\gamma$ -Fe<sub>2</sub>O<sub>3</sub> is contacted with a finely-divided carbonaceous reductant at a temperature in the range of from 350° C. to 540° C., comprising mixing and contacting said finely-divided  $\gamma$ -Fe<sub>2</sub>O<sub>3</sub> with reducing gas to fluidize said  $\gamma$ -Fe<sub>2</sub>O<sub>3</sub>, introducing the resultant mixture into the top of a reduction zone within a vertical furnace-like closed reduction chamber at a plurality of points distributed over the horizontal area of the reduction zone, mixing finely-divided carbonaceous reductant with reducing gas, intermittently introducing the resultant second mixture into said reduction zone in more than one horizontal area thereof by blowing said second mixture in a vertical upward direction from a plurality of points distributed over each of said horizontal areas, the points on each of said areas being disposed below and staggered from the points on the area immediately above, whereby said first mixture falling down through said reduction zone is suspended above each of said horizontal areas by the upward blowing second mixture and dropped to the next lower horizontal area by intermittently stopping the flow of said second mixture at each of said areas, thereby

intimately contacting said first mixture with said second mixture and slowly transporting said first mixture continuously from the top of said reduction zone to the bottom of said reduction zone, and cooling the reduced material at the lower part of said reduction zone within the vertical furnace-like closed chamber to a temperature below 100° C.

2. A process for the production of pure iron from brown magnetic iron oxide,  $\gamma$ -Fe<sub>2</sub>O<sub>3</sub>, and another iron composition selected from the group consisting of hematite, magnetite and mixtures thereof, in which finely-divided  $\gamma$ -Fe<sub>2</sub>O<sub>3</sub> and said other iron composition in finely-divided form are contacted with a finely divided carbonaceous reductant, comprising mixing said finely-divided  $\gamma$ -Fe<sub>2</sub>O<sub>3</sub> with said other finely divided iron composition to twice the weight of  $\gamma$ -Fe<sub>2</sub>O<sub>3</sub>, mixing and contacting said mixture with reducing gas to fluidize said mixture, introducing the resultant fluidized mixture into the top of a reduction zone within a vertical furnace-like closed reduction chamber at a plurality of points distributed over the horizontal area of this reduction zone, mixing finely-divided carbonaceous reductant with reducing gas, intermittently introducing the resultant second fluidized mixture into said reduction zone in more than one horizontal area thereof by blowing said second fluidized mixture in vertical upward direction from a plurality of points distributed over each of said horizontal areas, the points on each of said areas being disposed below and staggered from the points on the area immediately above, whereby said first fluidized mixture falling down through said reduction zone is suspended above each of said horizontal areas by the upward blowing second fluidized mixture and dropped to the next lower horizontal area by intermittently stopping the flow of said second fluidized mixture at each of said areas, thereby intimately contacting said first fluidized mixture with said second fluidized mixture and slowly transporting said first fluidized mixture continuously from the top of said reduction zone to the bottom of said reduction zone, and cooling the reduced material at the lower part of said reduction zone within the vertical furnace-like closed chamber to a temperature below 100° C.

3. A process for the production of pure iron from brown magnetic iron oxide,  $\gamma$ -Fe<sub>2</sub>O<sub>3</sub>, and another iron composition from the group consisting of hematite, magnetite and mixtures thereof, in which finely-divided  $\gamma$ -Fe<sub>2</sub>O<sub>3</sub> and said other iron composition in finely-divided form are contacted with a finely-divided carbonaceous reductant, comprising mixing said finely-divided  $\gamma$ -Fe<sub>2</sub>O<sub>3</sub> with said other finely-divided iron composition up to twice the weight of  $\gamma$ -Fe<sub>2</sub>O<sub>3</sub> and finely-divided carbonaceous reductant, pelletizing said mixture at a temperature below 200° C., mixing and contacting said pelletized mixture with reducing gas to fluidize said mixture, introducing said fluidized mixture into the top of a reduction zone within a vertical furnace-like closed reduction chamber at a plurality of points distributed over the horizontal area of this reduction zone, mixing finely-divided carbonaceous reductant with reducing gas, intermittently introducing the resultant second fluidized mixture into said reduction zone in more than one horizontal area thereof by blowing said second fluidized mixture in vertical upward direction from a plurality of points distributed over each of said horizontal areas, the points on each of said areas being disposed below and staggered from the points on the area immediately above, whereby said first fluidized mixture falling down through said reduction zone is suspended above each of said horizontal areas by the upward blowing second fluidized mixture and dropped to the next lower horizontal area by intermittently stopping the flow of said second fluidized mixture at each of said areas, thereby intimately contacting said first fluidized mixture with said second fluidized mixture and slowly transporting said first fluidized mixture continuously from the top of said reduction zone to the

bottom of said reduction zone, and cooling the reduced material at the lower part of said reduction zone within the vertical furnace-like closed chamber to a temperature below 100° C.

## References Cited in the file of this patent

## UNITED STATES PATENTS

171,812 Hunter Jan. 4, 1876

|           |                 |               |
|-----------|-----------------|---------------|
| 1,829,124 | Wilson          | Oct. 27, 1931 |
| 2,333,111 | Lykken          | Nov. 2, 1943  |
| 2,389,133 | Brassert et al. | Nov. 20, 1945 |
| 2,598,796 | Hulthen         | June 3, 1952  |
| 2,716,601 | Crowley         | Aug. 30, 1955 |
| 2,742,352 | Gilliland       | Apr. 17, 1956 |
| 2,742,354 | Ogorzaly        | Apr. 17, 1956 |
| 2,747,988 | Von Haken       | May 29, 1956  |